

## UNITED STATES PATENT OFFICE

1,969,479

## METHOD OF PRODUCING COLOR PHOTOGRAPHIC IMAGES BY DEVELOPMENT

Merrill W. Seymour, Irondequoit, N. Y., assignor  
to Eastman Kodak Company, Rochester, N. Y.,  
a corporation of New York

No Drawing. Application May 11, 1931,  
Serial No. 536,659

6 Claims. (Cl. 95—88)

This invention relates to photographic developers capable of producing directly colored images.

Developers have been known which are capable of developing silver halide salts directly to colored compounds by means of a combination between an oxidation product of the developer and another substance added to the developer, or by the oxidation of the developer itself by the silver halide to a colored substance.

I have found a class of organic substances very useful in processes of this sort. These substances are completed or partial condensation products of a hydrazine with an acyl acetic acid ester. The pyrazolones are examples of these products which are particularly useful. These substances are made by condensing the corresponding hydrazines with  $\beta$  keto-acid esters, such as aceto-acetic ethyl ester, or with  $\beta$  aldehyde acids.

In carrying out these condensations a hydrazine may be used to react with, for example, formyl acetic acid esters, aceto acetic acid esters, or benzoyl acetic acid esters. Intermediate products, particularly the aryl hydrazones of these acyl acetic acid esters, are useful in place of the pyrazolones.

Pyrazolones that I have found particularly useful are the following: 1-phenyl-3-methyl-5-pyrazolone, 1-p-nitrophenyl-3-methyl-5-pyrazolone, 1- $\alpha$ -naphthyl-3-methyl-5-pyrazolone, 1-p-bromophenyl-3-methyl-5-pyrazolone, pyrazolone (unsubstituted), 3-phenyl-pyrazolone.

These substances and any others which I may use are distinguished from other pyrazolones previously mentioned as follows. They are all characterized by the fact that at the 4 position there is always an active methylene group. This statement is made clearer by consideration of the following formula, which is general for the substances under consideration.



The commonly accepted nomenclature is used and the positions from 1 to 5 are numbered as shown. X and Y may be either hydrogen, an

aryl group or an alkyl group. Preferably not both X and Y are hydrogen. It is seen that the 4 position is occupied by the methylene ( $-\text{CH}_2-$ ) group. This is the particular characteristic of all of the compounds which I use.

An example of the use of an intermediate is p-nitro-phenyl-hydrazone of aceto-acetic ethyl ester, an intermediate product in the formation of 1-p-nitro-phenyl-3-methyl-5-pyrazolone.

The pyrazolones and hydrazones described react in the developer with the oxidation products of p-phenylene diamine or its alkyl substituted compounds such as p-amino-diethylaniline or p-amino-dimethylaniline to form insoluble dyes. Although the p-phenylene diamine may be, and is preferably alkyl substituted, one of the amino groups must be unsubstituted. The other may have one or two alkyl substituents.

An example of the use of the invention follows. The following developer is made up:

## EXAMPLE I

## Solution A

|                                |           |    |
|--------------------------------|-----------|----|
| 1-phenyl-3-methyl-5-pyrazolone | 0.5 grams | 75 |
| Acetone                        | 10. cc.   |    |

## Solution B

|                                   |           |    |
|-----------------------------------|-----------|----|
| p-amino-dimethylaniline           | 0.5 grams |    |
| Sodium carbonate 10% aqueous sol. | 75. cc.   | 80 |
| Water                             | 175. cc.  |    |

For use add Solution A to Solution B.

The exposed plate or film is developed in this developer, which gives a certain amount of reduced silver image, together with an image of a complex compound having a red or rose color. The silver is removed by means of well-known bleaching solutions such as Farmer's reducer or a bleach consisting of potassium ferricyanide and potassium bromide. The Farmer's reducer is preferably used as two separate solutions, one containing the potassium ferricyanide and the other the hypo. With the ferricyanide-bromide type of bleach it is necessary to follow the treatment with fixing in hypo to remove soluble silver salts.

It is, of course, requisite that the bleach used should not affect the colored image. This requirement will exclude the use of certain types

of bleaching solutions though a number are available and useful.

Another example of a suitable developer is the following:

5

## EXAMPLE II

|                                           |          |
|-------------------------------------------|----------|
| p-nitrophenyl hydrazone of acetoacetic    |          |
| ethyl ester                               | 0.5 gm.  |
| Sodium carbonate, 10% solution            | 75. cc.  |
| 10 p-amino dimethyl aniline hydrochloride | 0.1 gm.  |
| Acetone                                   | 40. cc.  |
| Water to                                  | 200. cc. |

15 As before, the film is developed in this developer and the silver is bleached out with one of the solutions mentioned. This yields an image of a peculiar shade of rose color.

A third suitable developer is

20

## EXAMPLE III

|                                                                               |          |
|-------------------------------------------------------------------------------|----------|
| Sodium carbonate 10% aqueous solution                                         | 30. cc.  |
| Sodium sulfite anhydrous                                                      | 1. gm.   |
| 25 p-amino dimethyl aniline hydrochloride                                     | 0.2 gm.  |
| 1-phenyl-3-methyl - 5 - pyrazolone 0.2 grams dissolved in ethyl alcohol 95% - | 10. cc.  |
| Potassium bromide 10%                                                         | 0.2 cc.  |
| Water to                                                                      | 100. cc. |

30 The components of a developer of the type I have described may be combined as illustrated in the foregoing examples and applied as a complete color developing solution to an exposed 35 silver halide layer, or one of the essential components which react to form the colored substance may be incorporated into a photographic emulsion, as by adsorption to the silver halide grains, and the other components, including preferably, the reducing agent, may be applied in 40 solution after exposure.

As an example of the use of these color forming substances adsorbed to silver halide salts, I may make an emulsion of silver bromide containing 45 a condensation product of a hydrazine with an acyl acetic acid ester. Particularly useful products of this kind are the pyrazolones. Such an emulsion is coated on a suitable support, dried, and exposed in the usual manner, as for example, 50 to a color separation image. It is then developed in a p-phenylene-diamine as described and the coupling action of the oxidation product of the developer with the pyrazolone or hydrazone

takes place in the presence of the image which is being developed in exactly the same way as previously described.

In mentioning processes of this kind, it is understood that I do not limit myself to cases in which the color former is truly adsorbed, as I contemplate the use of such color formers in any process where they are adsorbed, absorbed, or merely occur in close association with the sensitive salts.

It has previously been suggested to use a pyrazolone in a photographic developer in place of reducing agents such as methyl paraamino phenol sulphate (Elon). It is to be noted that I do not use the pyrazolones I have mentioned in this way, but only as substances which may couple with another substance on development to form a colored substance. This forms the basis of a quite different process.

What I claim is:

1. A photographic developer containing a condensation product of phenyl hydrazine with an acyl acetic acid ester, the condensation product being selected from the group consisting of a pyrazolone having an active methylene group in the 4 position and the hydrazone of the acyl acetic acid ester, the developer containing also a substance which on development reacts with said condensation product to produce a colored image.

2. A photographic developer containing p-phenylene diamine and a pyrazolone having an active methylene group in the 4 position.

3. A photographic developer containing a pyrazolone having an active methylene group in the 4 position and a substance which on development reacts with said pyrazolone to produce a colored image.

4. A photographic developer containing p-phenylene diamine and a condensation product of phenyl hydrazine with an acyl acetic acid ester, the condensation product being selected from the group consisting of a pyrazolone having an active methylene group in the 4 position and the hydrazone of the acyl acetic acid ester.

5. A photographic developer containing p-phenylene diamine and a hydrazone of an acyl acetic acid ester.

6. A photographic developer containing a hydrazone of an acyl acetic acid ester and a substance which on development reacts with said hydrazone to produce a colored image.

MERRILL W. SEYMOUR.

55

130

60

135

65

140

70

145

75

150